

Nov. 3, 1970

D. B. CALDWELL

3,537,717

DAMPED SKI AND METHOD OF MAKING

Filed Nov. 29, 1968



FIG. 1



FIG. 2



FIG. 3

INVENTOR.  
**DONALD B. CALDWELL**  
BY Kinney, Alexander,  
Selly, Sledick & De La Hunt  
ATTORNEYS

## 1

3,537,717

**DAMPED SKI AND METHOD OF MAKING**  
Donald B. Caldwell, East Oakdale, Minn., assignor to  
Minnesota Mining and Manufacturing Company, St.  
Paul, Minn., a corporation of Delaware

Filed Nov. 29, 1968, Ser. No. 780,088  
Int. Cl. A63c 5/12

U.S. CL. 280—11.13

4 Claims

### ABSTRACT OF THE DISCLOSURE

Ski flutter is greatly reduced and maneuverability enhanced by sandwiching a viscoelastic layer (formed, e.g., from certain acrylic copolymers) between the upper surface of the ski and a stretch-resistant constraining layer (e.g., aluminum sheet).

### BACKGROUND OF THE INVENTION

This invention relates to skis and to methods of improving the performance thereof.

Prior to the last three decades, virtually all skis were made of wood. Relatively few woods, however, have the strength, wear resistance, ability to retain camber and flexibility needed to make good skis. Even with suitable woods, great care must be exercised in selection, since any defect will alter the performance characteristics and may actually render the ski dangerous to use. Further, no matter what wood is chosen, it is difficult to form two skis having identical physical properties. It is not surprising, then, that the mass production of matched wood skis of high quality has never been possible.

In the last quarter century a great deal of effort has been devoted to the manufacture of skis having a shell or skeleton of metal and/or reinforced plastics, the interior core typically being filled with wood blocks, foamed plastic or other material which provides compressive strength. Such skis are uniform, predictable, and have significantly greater wear resistance and useful life. On the other hand, such skis have a somewhat different "feel" than wooden skis, typically displaying a greater degree of flutter, or vibration, particularly when used on steep or icy slopes, or when making sharp turns. Although it has been felt that flutter was a minor consequence, attempts have been made to damp skis by modifying their internal construction, seeking to make their performance more closely resemble that of wooden skis. Prior to the present invention, however, such attempts have been at best only modestly successful.

### SUMMARY

The present invention provides an improved ski construction in which mass-produced skis can be made to have the "feel" and lack the flutter characteristic of wooden skis. The resultant product is one which combines the best physical attributes of both the earlier wooden skis and the modern carefully constructed synthetic products. If desired, skis can be initially manufactured in accordance with the invention, but it is almost equally satisfactory to modify a pair of commercial skis to incorporate the features of the invention, very little time or effort being required. A surprising and unexpected feature of the modified ski construction is a noticeably enhanced maneuverability, as is particularly manifested by increased speed in slalom competition.

## 2

Skis made in accordance with the present invention have as their uppermost surface a stretch-resistant constraining layer such as aluminum or stainless steel sheet, glass filament-reinforced plastic, etc. Interposed between the lower surface of the constraining layer and the underlying rigid constructional face of the ski is a viscoelastic layer which has a thickness of at least 0.015 inch (about 0.4 mm.), a glass transition temperature in the range of  $-55^{\circ}\text{C}$ . to  $-85^{\circ}\text{C}$ , and, at temperatures throughout the range of  $-25^{\circ}\text{C}$ . to  $+5^{\circ}\text{C}$ . and frequencies of 10–20 Hz., a loss tangent value of at least 0.5 (preferably at least 0.7) and a dynamic shear modulus in the range of 0.7–700 kg./cm.<sup>2</sup>. The constraining layer and the viscoelastic layer are further selected so that the dynamic stretching stiffness of the former, measured in force per unit width, is significantly higher than (preferably at least 10 times as great as), the dynamic shear stiffness of the latter, measured in force per unit volume in the foregoing temperature and frequency ranges, all measurements being in c.g.s. units.

20 A commercial ski is conveniently modified with the aid of a strip of damping material formed by applying a viscoelastic layer to one face of a suitable constraining layer (e.g., thin aluminum sheet) and then adhering the viscoelastic layer to the upper surface of the ski. The entire upper surface of the ski may be provided with the strip of damping material, although satisfactory results are obtained by applying the damping material in a strip extending longitudinally from the bindings to the front 25 touchdown point of the ski. For men's skis which are at least 78 inches (approximately 200 cm.) long, a 32-inch (approximately 81 cm.) long damping strip has been found extremely suitable. Preferably the viscoelastic layer has aggressive pressure-sensitive adhesive characteristics, facilitating attachment of the damping strip and permitting removal if and when desired. It is also contemplated, however, to employ a viscoelastic layer which lacks adequate adhesiveness, a separate pressure-sensitive or other adhesive being used to bond the viscoelastic layer 30 to the upper surface.

35 Suitable viscoelastic materials may be based on polyisobutylene. Particularly preferred, however, are copolymers of alkyl acrylate and one or more copolymerizable acrylic monomers such as acrylic acid, methacrylic acid, acrylonitrile, methacrylonitrile, acrylamide and methacrylamide. The alkyl acrylate may be a single monomer having about 6–10 carbon atoms in its alkyl group which is not highly branched, i.e., more than half of the alkyl carbon atoms are in a straight chain terminating at the 40 oxygen bridge. Where the alkyl acrylate is a mixture of monomers, their alkyl groups should have an average of about 6–10 carbons, and less than half of the alkyl groups should be highly branched. Because of their age-resistance, affinity for metals, adhesion characteristics and viscoelastic properties at the range of temperatures 45 encountered, copolymers containing 90–97% isoctyl acrylate and correspondingly 10–3% acrylic acid are especially preferred.

50 Depending on the degree of damping which is sought and the personal preference of the user, the strip of damping material can be the same width as the ski; alternatively, one or more strips of lesser width, preferably arranged symmetrically can be applied. Likewise, a plurality of damping strips can be superposed and adhered 55 to the ski; in such case, the width of each strip may be 60

the same or, if desired, upper strips may be narrower than lower strips. It is also apparent that for sophisticated skiers, the degree of damping may be tailored to the individual or the snow conditions, damping strips being added or removed as desired. Generally, however, it has been found that a ski which has been damped is more satisfactory to an individual for all skiing conditions.

In order to demonstrate the effectiveness of the present invention in reducing ski flutter, a test has been devised to measure the duration of vibrations set up in a ski. In this test, the rear portion of a ski (i.e., that portion lying more than  $3\frac{1}{2}$  inches (about 9 cm.) behind the mid point of the ski) is held in a massive rigid clamp. A light weight vibration pickup is then attached approximately 6 inches (15 cm.) to the rear of the front touchdown point. The ski is then set into vibration by lightly plucking the tip, vibration thereafter continuing at the resonant frequency of the ski (which is almost always in the range of 10-15 Hz.) and gradually dying away. The output of the vibration pickup is fed into a recorder having a strip chart moved beneath a marking pen at a speed of 25 mm. per second. From the chart, the resonant frequency is calculated and the average height ratio of several succeeding peaks measured, thereby obtaining the average peak to peak decrement ratio. The formula for vibration decay rate,  $D$ , expressed in decibels per second, is  $D=8.68 K^1$ , where  $K$  is  $\log_e$  of the amplitude decrement ratio per second (i.e.,  $\log_e$  of the product of frequency in Hz. and the average decrement ratio). A typical decay rate for a wooden ski is about 15 db/sec.; the vibration decay rates for conventional non-wooden skis are usually in the range of 2-5 db/sec., with a few approaching 15 db/sec. It has been found that, regardless of the nature of the ski to which damping strips made in accordance with this invention are applied, the decay rate can easily be increased by 10-20 decibels per second. If desired, of course, the dimensions of the strip can be varied to achieve a greater or lesser degree of damping.

When a ski is modified in accordance with this invention by applying a strip of damping material to the upper surface, the strip is preferably chosen so that the weight increase is held to a minimum. In evaluating the effectiveness of a given damping strip, it has been found useful to employ the "damping index," an arbitrarily selected parameter which is defined as the vibration decay rate increase in db/sec. (compared to a bare ski) divided by the weight of the damping strip in grams. It is preferred that the weight increase does not exceed 200 grams and that the damping index be at least about 0.1.

It is also preferred that the thickness of the entire damping strip be held to as low a caliper as feasible, the overall thickness preferably being no more than about 0.1 inch (2.5 mm.), not only to minimize weight but also to facilitate moving the ski sideways through snow. It has been found, however, that it is important for the overall thickness to be at least about 0.02 inch (0.5 mm.) if significant improvement is to be obtained. Satisfactory results have been achieved where the constraining layer is sheet aluminum having a thickness in the range of 0.015-0.050 inch (about 0.4-1.25 mm.) and the viscoelastic layer has a thickness of at least about 0.015 inch (about 0.4 mm.). Particularly good results are obtained with a 0.032-inch aluminum sheet (about 0.8 mm.) and a 0.025-inch (about 0.6 mm.) viscoelastic layer. If stainless steel is substituted for the aluminum, the constraining layer can be made thinner; the weight for comparable performance, however, is about the same.

#### BRIEF DESCRIPTION OF THE DRAWING

Understanding of the invention will be facilitated by reference to the accompanying drawing, in which:

FIG. 1 is a side elevational view showing one form of ski made in accordance with the invention;

FIG. 2 is a top view of a conventional ski modified in accordance with the present invention; and

FIG. 3 is an enlarged cross-sectional view of a portion of the ski shown in FIG. 2, taken along section lines 3-3.

#### DESCRIPTION OF PRESENTLY PREFERRED EMBODIMENTS

FIG. 1 depicts a ski 10 having a body portion 11, the lower surface of which has front touchdown 12 and rear touchdown 13. Damping strip 14 comprises constraining number 15 and viscoelastic layer 16, the latter being firmly adhered to the upper surface of body 11. Numeral 17 designates the general location where a ski boot (not shown) is attached when ski 10 is used.

FIGS. 2 and 3 depict a ski 10a having body 11a, with front touchdown 12a and rear touchdown 13a. To the upper forward surface of body 11a are attached damping strips 14a, each individually similar to damping strip 14 as shown in FIG. 1, comprising constraining member 15a and viscoelastic layer 16a. Damping strips 14a extend longitudinally from approximately the forward portion of boot location 17a to front touchdown 12a.

Understanding of the invention will be further enhanced by referring to the following illustrative but non-limitative examples, in which all parts are by weight unless otherwise noted.

#### EXAMPLES

A glass fiber-filled 95.5:4.5 iso-octylacrylate: acrylic acid copolymer, for use as a viscoelastic material in practicing the invention was prepared in accordance with Example 1 of Kalleberg and Turner U.S. Pat. 3,062,683 and knife-coated on a glassine-kraft paper carrier web having a silicone-treated release surface on both sides. The coated carrier web was dried in an air-circulating oven at about 100° C. for 2 minutes, 155° C. for 3 minutes and finally about 130° C. for 6 minutes to provide a dried coating about 1 mil (25 microns) thick, whereupon the coated carrier web was wound upon itself in roll form for storage. To insure that the coating was sufficiently dry, a small piece of the coating was weighed and then conditioned for two hours at 25° C. and 30% relative humidity and reweighed. No loss in weight indicated that the coating was substantially free from volatile material and thus could be used for a viscoelastic layer. Loss of weight during the conditioning period would have indicated the presence of trapped volatiles which could result in undesirable change in damping performance during use. The loss tangent and dynamic shear modulus, measured with apparatus such as that described by E. J. Fitzgerald in The Physical Review, vol. 108, pp. 690 et seq. (1957) and extrapolated by conventional methods, were found to be as set forth below:

|                    | Frequency,<br>Hz. | Loss<br>tangent <sup>1</sup> | Dynamic<br>shear<br>modulus,<br>kg./cm. <sup>2</sup> |
|--------------------|-------------------|------------------------------|------------------------------------------------------|
| Temperature, ° C.: |                   |                              |                                                      |
| +5                 | 10                | 0.83                         | 0.85                                                 |
| +5                 | 20                | 0.90                         | 1.1                                                  |
| -23                | 10                | 1.8                          | 8.8                                                  |
| -23                | 20                | 1.6                          | 13.8                                                 |

<sup>1</sup> The glass fibers have no appreciable effect on these values and can, if desired, be omitted; the fibers serve primarily to prevent any tendency of the viscoelastic material to ooze.

Dynamic shear stiffness is calculated for a given viscoelastic layer by dividing the dynamic shear modulus by the stiffness. Glass transition temperature, determined by refractive index measurements, was -71° C.

Damping strips were prepared as follows: A 30-inch diameter metal roll was wrapped with 5-mil (0.127 mm.) biaxially-oriented and heat-set polyethylene terephthalate (polyester) film. The roll was then rotated while the coated carrier web was pressed against the film by a spring-loaded

<sup>1</sup> Cf., e.g., Greiger and Hamme Laboratories Report No. U.S. Navy 1 (April 1961), entitled "The Concept of Damping of Structureborne Sound and Vibration for Noise Control."

laminating roll to transfer the copolymer coating to the polyester film, and the carrier web was stripped away. This was continued until the successive convolutions of the copolymer coating reached a total thickness of 25 mils (approximately 0.6 mm.), the carrier web being allowed to contact the outermost convolution of the coating. The temporary laminate of the liner, copolymer coating and polyester film were then slit parallel to the axis of the roll, removed therefrom, chilled to about 5° C. and the polyester film removed. The coated liner was then placed on a table, coated side up, several widths of 32-inch long 7075T6 aluminum strips, ranging from 0.016 to 0.040 inch (approximately 0.4 to 1 mm.) thick, placed on the coated surface, and the damping material and liner trimmed to size with a razor blade. (The Young's modulus for 7075T6 aluminum strips is approximately 7,000,000 kg./cm.<sup>2</sup>; stretching stiffness is calculated as the product of

5 From the foregoing table it is observed that a 0.016" (0.41 mm.) aluminum restraining layer is not quick enough to obtain optimum results. It is inferred that it stretches slightly, thereby diminishing the effect of the viscoelastic material. The 0.032" (0.81 mm.) aluminum layer, however, is eminently satisfactory and offers a clear cut weight savings over the 0.040" (1.02 mm.).

10 It was also concluded that a 0.025" (0.64 mm.) layer of viscoelastic material represented a good compromise of performance characteristics, thinner layers being more prone to shock loose and thicker layers offering, at best, no more than nominal improvements.

15 The following table summarizes the effect of adding damping strips [32" (81 cm.) long, full ski width, 0.032" (0.81 mm.) 7075T6 aluminum, 0.025" (1 mm.) 95.5:4.5 isoocetyl acrylate: acrylic acid copolymer viscoelastic adhesive] to several types of skis.

TABLE II

|                              |                                  | Decay rates, db/sec. |                    |          |
|------------------------------|----------------------------------|----------------------|--------------------|----------|
| Ski construction             | Manufacturer and model           | Bare ski             | With damping strip | Increase |
| Metal                        | Hart "Javelin"                   | 2.2                  | 19.8               | 17.6     |
| Do                           | Hart "Camaro"                    | 2.6                  | 19.4               | 16.8     |
| Do                           | Head "360"                       | 2.9                  | 18.7               | 15.8     |
| Do                           | Head "GS"                        | 3.9                  | 16.6               | 12.7     |
| Glass fiber-reinforced resin | G.M.P. Sports LTD, "Tony Sailer" | 2.6                  | 18.0               | 15.4     |
| Do                           | Kastle "CPM-70"                  | 3.5                  | 18.6               | 15.1     |
| Do                           | Rossignol "Strato"               | 4.2                  | 18.4               | 14.2     |
| Do                           | Dynamic "VR-17"                  | 4.7                  | 19.2               | 14.5     |
| Do                           | Kneissl "Black Star"             | 13.1                 | 28.0               | 13.9     |

Young's modulus times thickness. The stretching stiffnesses of 0.4-mm. and 1-mm. aluminum are thus respectively about 280,000 kg./cm. and 700,000 kg./cm.)

35 Other damping strips were prepared in the manner just described, varying the number of convolutions applied to the drum to attain several thicknesses of damping material. The several damping strips, each 32 inches (approximately 81 cm.) long, were then applied to the forward part of two different metal skis—a 6'9" (206 cm.) Kastle "Metall" and a 7' (213 cm.) Northland "Golden Jet"—which were then checked for rate of vibration decay, using the test procedure previously described. Results obtained using damping strips the same width as the ski are tabulated below:

TABLE I

| Temper-<br>ature, ° C. | Ski                   | Viscoelastic<br>layer thick-<br>ness, mm. | Constraint<br>layer thick-<br>ness, mm. | Decay<br>rate,<br>db/sec. | Decay<br>rate,<br>db/sec. | Damping<br>weight,<br>grams | Damping<br>index |
|------------------------|-----------------------|-------------------------------------------|-----------------------------------------|---------------------------|---------------------------|-----------------------------|------------------|
| Example:               |                       |                                           |                                         |                           |                           |                             |                  |
| Control                | minus 7 "Metall"      |                                           |                                         | 9.6                       |                           |                             |                  |
| 1                      | minus 7 do            | 0.38                                      | 0.41                                    | 17.7                      | 8.1                       | 85.0                        | 0.095            |
| 2                      | minus 7 do            | 0.38                                      | 0.81                                    | 30.3                      | 20.7                      | 151.3                       | 0.137            |
| 3                      | minus 7 do            | 0.64                                      | 0.41                                    | 21.8                      | 12.2                      | 96.1                        | 0.127            |
| 4                      | minus 7 do            | 0.64                                      | 0.81                                    | 28.9                      | 19.3                      | 164.2                       | 0.118            |
| 5                      | minus 7 do            | 1.27                                      | 0.41                                    | 20.8                      | 11.2                      | 128.9                       | 0.087            |
| 6                      | minus 7 do            | 1.27                                      | 0.81                                    | 30.0                      | 20.4                      | 197.0                       | 0.104            |
| 7                      | minus 7 do            | 1.27                                      | 1.02                                    | 34.2                      | 24.6                      | 242.1                       | 0.102            |
| Control                | minus 7 "Golden Jet"  |                                           |                                         | 3.6                       |                           |                             |                  |
| 1a                     | minus 7 do            | 0.38                                      | 0.41                                    | 12.3                      | 8.7                       | 85.0                        | 0.102            |
| 2a                     | minus 7 do            | 0.38                                      | 0.81                                    | 20.0                      | 16.4                      | 151.3                       | 0.108            |
| 3a                     | minus 7 do            | 0.64                                      | 0.41                                    | 13.1                      | 9.5                       | 96.1                        | 0.099            |
| 4a                     | minus 7 do            | 0.64                                      | 0.81                                    | 23.0                      | 19.4                      | 164.2                       | 0.118            |
| 5a                     | minus 7 do            | 1.27                                      | 0.41                                    | 13.4                      | 10.8                      | 128.9                       | 0.084            |
| 6a                     | minus 7 do            | 1.27                                      | 0.81                                    | 25.8                      | 22.2                      | 197.0                       | 0.113            |
| 7a                     | minus 7 do            | 1.27                                      | 1.02                                    | 23.4                      | 19.8                      | 242.1                       | 0.082            |
| Control                | minus 13 "Metall"     |                                           |                                         | 8.8                       |                           |                             |                  |
| 1                      | minus 13 do           | 0.38                                      | 0.41                                    | 16.3                      | 7.5                       | 85.4                        | 0.088            |
| 2                      | minus 13 do           | 0.38                                      | 0.81                                    | 27.1                      | 18.3                      | 151.2                       | 0.121            |
| 3                      | minus 13 do           | 0.64                                      | 0.41                                    | 17.2                      | 8.4                       | 96.2                        | 0.087            |
| 4                      | minus 13 do           | 0.64                                      | 0.81                                    | 27.5                      | 18.7                      | 164.1                       | 0.114            |
| 5                      | minus 13 do           | 1.27                                      | 0.41                                    | 20.1                      | 12.3                      | 128.7                       | 0.098            |
| 6                      | minus 13 do           | 1.27                                      | 0.81                                    | 29.4                      | 20.6                      | 197.0                       | 0.105            |
| Control                | minus 13 "Golden Jet" |                                           |                                         | 3.9                       |                           |                             |                  |
| 1a                     | minus 13 do           | 0.38                                      | 0.41                                    | 10.9                      | 7.0                       | 85.4                        | 0.082            |
| 2a                     | minus 13 do           | 0.38                                      | 0.81                                    | 19.8                      | 15.9                      | 151.2                       | 0.105            |
| 3a                     | minus 13 do           | 0.64                                      | 0.41                                    | 13.1                      | 9.2                       | 96.2                        | 0.096            |
| 4a                     | minus 13 do           | 0.64                                      | 0.81                                    | 21.2                      | 17.3                      | 164.0                       | 0.116            |
| 5a                     | minus 13 do           | 1.27                                      | 0.41                                    | 15.9                      | 12.0                      | 128.7                       | 0.093            |
| 6a                     | minus 13 do           | 1.27                                      | 0.81                                    | 24.2                      | 20.3                      | 197.0                       | 0.103            |
| Control                | minus 23 "Metall"     |                                           |                                         | 7.7                       |                           |                             |                  |
| 1                      | minus 23 do           | 0.38                                      | 0.81                                    | 20.8                      | 13.1                      | 151.6                       | 0.086            |
| 2                      | minus 23 do           | 0.64                                      | 0.81                                    | 21.2                      | 13.5                      | 166.3                       | 0.081            |
| Control                | minus 23 "Golden Jet" |                                           |                                         | 4.6                       |                           |                             |                  |
| 2a                     | minus 23 do           | 0.38                                      | 0.81                                    | 16.4                      | 11.8                      | 151.6                       | 0.078            |
| 4a                     | minus 23 do           | 0.64                                      | 0.81                                    | 17.7                      | 13.1                      | 166.3                       | 0.079            |

width are likewise effective. The skis tested were the same as those listed in Table I, the constraint layer being 0.032-inch (0.81 mm.) aluminum in all cases.

down point, at least one elongated strip of a damping material comprising in combination:

a viscoelastic layer adhered over said upper surface of

TABLE III

| Damping strip width, cm. | Temper-ature, °C. | Ski              | Visco-elastic layer thickness, mm. | Decay rate, db/sec. | Decay rate increase, db/sec. | Damping weight, grams | Damping index |
|--------------------------|-------------------|------------------|------------------------------------|---------------------|------------------------------|-----------------------|---------------|
| <b>Example:</b>          |                   |                  |                                    |                     |                              |                       |               |
| Control                  |                   | -7 "Metall"      | 9.6                                |                     |                              |                       |               |
| 8                        | 5.1               | -7 do            | 0.38                               | 21.2                | 11.6                         | 108.7                 | 0.107         |
| 9                        | 5.1               | -7 do            | 0.64                               | 24.5                | 14.9                         | 116.9                 | 0.127         |
| 10                       | 5.1               | -7 do            | 1.27                               | 24.2                | 14.6                         | 141.0                 | 0.103         |
| 11                       | 2.5               | -7 do            | 0.38                               | 18.2                | 8.6                          | 53.9                  | 0.159         |
| 12                       | 2.5               | -7 do            | 0.64                               | 16.3                | 6.7                          | 58.9                  | 0.114         |
| 13                       | 2.5               | -7 do            | 1.27                               | 17.9                | 8.3                          | 70.7                  | 0.117         |
| Control                  |                   | -7 "Golden Jet"  | 3.6                                |                     |                              |                       |               |
| 8a                       | 5.1               | -7 do            | 0.38                               | 16.4                | 12.8                         | 108.7                 | 0.118         |
| 9a                       | 5.1               | -7 do            | 0.64                               | 17.4                | 13.8                         | 116.9                 | 0.118         |
| 10a                      | 5.1               | -7 do            | 1.27                               | 18.0                | 14.4                         | 141.0                 | 0.102         |
| 11a                      | 2.5               | -7 do            | 0.38                               | 12.0                | 8.4                          | 53.9                  | 0.156         |
| 12a                      | 2.5               | -7 do            | 0.64                               | 12.3                | 8.7                          | 58.9                  | 0.148         |
| 13a                      | 2.5               | -7 do            | 1.27                               | 14.6                | 11.0                         | 70.7                  | 0.156         |
| Control                  |                   | -13 "Metall"     | 8.8                                |                     |                              |                       |               |
| 8                        | 5.1               | -13 do           | 0.38                               | 25.4                | 16.6                         | 108.7                 | 0.153         |
| 9                        | 5.1               | -13 do           | 0.64                               | 29.0                | 20.2                         | 116.9                 | 0.173         |
| 10                       | 5.1               | -13 do           | 1.27                               | 29.4                | 20.6                         | 141                   | 0.146         |
| Control                  |                   | -13 do           | 3.1                                |                     |                              |                       |               |
| 11                       | 2.5               | -13 do           | 0.38                               | 13.9                | 10.8                         | 54                    | 0.200         |
| 12                       | 2.5               | -13 do           | 0.64                               | 14.3                | 11.2                         | 58.8                  | 0.190         |
| 13                       | 2.5               | -13 do           | 1.27                               | 14.7                | 11.6                         | 70.7                  | 0.164         |
| 8a                       | 5.1               | -13 "Golden Jet" | 0.38                               | 17.8                | 14.7                         | 108.7                 | 0.135         |
| 9a                       | 5.1               | -13 do           | 0.64                               | 17.6                | 14.5                         | 116.9                 | 0.124         |
| 10a                      | 5.1               | -13 do           | 1.27                               | 19.8                | 16.7                         | 141                   | 0.119         |
| 11a                      | 2.5               | -13 do           | 0.38                               | 9.2                 | 6.1                          | 54                    | 0.113         |
| 12a                      | 2.5               | -13 do           | 0.64                               | 10.3                | 7.2                          | 58.8                  | 0.122         |
| 13a                      | 2.5               | -13 do           | 1.27                               | 13.3                | 10.2                         | 70.7                  | 0.144         |
| Control                  |                   | -23 "Metall"     | 7.7                                |                     |                              |                       |               |
| 8                        | 5.1               | -23 do           | 0.38                               | 20.2                | 12.5                         | 108.5                 | 0.115         |
| 9                        | 5.1               | -23 do           | 0.64                               | 22.1                | 14.4                         | 118.6                 | 0.121         |
| Control                  |                   | -23 "Golden Jet" | 4.6                                |                     |                              |                       |               |
| 8a                       | 5.1               | -23 do           | 0.38                               | 13.6                | 9.0                          | 108.5                 | 0.083         |
| 9a                       | 5.1               | -23 do           | 0.64                               | 16.3                | 11.7                         | 118.6                 | 0.099         |

What I claim is:

1. The method of reducing the normal tendency of a ski to chatter and vibrate on rough or icy substrates, comprising applying to the upper surface of said ski, in an area lying between the bindings and a touchdown point, at least one strip of a damping material comprising in combination:

a stretch-resistant constraining layer bearing, on the face adjacent the ski surface,

a viscoelastic layer, said viscoelastic layer having:

a glass transition temperature in the range of -55° C. to -85° C.,

a thickness of at least about 0.4 mm., and at temperatures throughout the range of -25° C. to +5° C. and at frequencies in the range of 10-20 Hz.,

a loss tangent of at least 0.5 and a dynamic shear modulus in the range of 0.7-700 kg./cm.<sup>2</sup>, the dynamic stretching stiffness of said constraining layer being significantly greater than the dynamic shear stiffness of said viscoelastic layer,

whereby the rate of vibration decay of said ski at its resonant frequency is significantly greater than its rate of vibration decay in the absence of said strip of damping material.

2. A ski having laminated to the upper surface thereof, in an area lying between the bindings and the front touch-

the ski, said viscoelastic layer having a thickness of at least about 0.4 mm. and at temperatures throughout the range of -25° C. to +5° C. and frequencies of 10-20 Hz., a loss tangent of at least 0.5 and a dynamic shear modulus in the range of 0.7-700 kg./cm.<sup>2</sup>,

40 a constraining layer laminated to the upper surface of the viscoelastic layer, said constraining layer having a dynamic stretching stiffness at least 10 times as great as the dynamic shear stiffness of said viscoelastic layer, the overall thickness of said damping material being 0.5-2.5 mm.

45 3. The ski of claim 2 wherein the viscoelastic layer has a loss tangent of at least 0.7.

4. The ski of claim 2 wherein the constraining layer is sheet aluminum having a thickness of 0.4-1.25 mm.

#### References Cited

##### UNITED STATES PATENTS

|           |         |          |
|-----------|---------|----------|
| 2,264,535 | 12/1941 | Klemm.   |
| 2,995,379 | 8/1961  | Head.    |
| 3,194,572 | 7/1965  | Fischer. |
| 3,300,226 | 1/1967  | Reed.    |
| 3,475,035 | 10/1969 | Nason.   |

60 LEO FRIAGLIA, Primary Examiner

M. L. SMITH, Assistant Examiner